

## UNITED STATES PATENT OFFICE

1,920,496

## INSULATING OR WALL BOARD PRODUCT

Carroll E. Carpenter, Western Springs, Ill., assignor, by mesne assignments, to United States Gypsum Company, Chicago, Ill., a Corporation of Illinois

No Drawing. Application August 23, 1928  
Serial No. 301,701

3 Claims. (Cl. 92—3)

My invention relates to fibre products and more especially to pulp or fibre insulating or wall board products or allied products.

Certain varieties of trees and plants have heretofore been employed in the manufacture of such pulp or fibre products with varying degrees of success. In the production of fibre or pulp products of this nature it is essential that the raw materials, when reduced to pulp form, shall have certain qualities largely measurable by the freeness of the pulp which will permit conversion to board at proper speeds on the various types of board forming machines available, and will, at the same time, give a product which, due to the cellular construction of the composite mass, will have the requisite degree of strength, flexibility, and insulating qualities. The product thus formed also should be such that it can be effectively sized or otherwise rendered water resistant during or after manufacture.

One object of my invention is to provide a pulp or fibre product which is well suited to the manufacture of relatively thick boards having a generally open or cellular structure, possessing a relatively high insulating value, as well as providing a board which is both light and strong with good nail-holding qualities and which is easy to cut and handle.

Another object of my invention is the provision of a fibre product having all or most of the above characteristics and made either from hard wood alone or from suitable admixtures of hard and soft woods. By the term "hard wood" it is meant to include such hard textured woods as are typified by the following group:

|             |                                    |
|-------------|------------------------------------|
| Oak (red)   | ( <i>Quercus borealis maxima</i> ) |
| Gum (black) | ( <i>Nyssa sylvatica</i> )         |
| Tupelo      | ( <i>Nyssa aquatica</i> )          |
| Hackberry   | ( <i>Celtis occidentalis</i> )     |
| 40 Magnolia | ( <i>Magnolia glauca</i> )         |
| Elm         | ( <i>Ulmus pubescens</i> )         |
| Maple       | ( <i>Acer rubrum</i> )             |
| Birch       | ( <i>Betula lutea</i> )            |
| 45 Beech    | ( <i>Fagus grandifolia</i> )       |

By the term "soft wood" it is meant to include such soft textured woods as are typified by the following group:

|                   |                               |
|-------------------|-------------------------------|
| 50 Cypress        | ( <i>Taxodium distichum</i> ) |
| Cottonwood        | ( <i>Populus deltoides</i> )  |
| Willow (longleaf) | ( <i>Salix fluvialis</i> )    |

Among the above mentioned varieties of trees, some are found in abundance particularly in the southern part of the United States and, while

readily accessible and relatively low in price, have not been heretofore usable for the purposes herein set forth nor has it been possible up to the present time to fully utilize their value in other ways. The problem, therefore, has been to render 60 these woods available for useful purposes. After carrying out a number of long and costly experiments, I have succeeded in the production of a product suitable for insulating and wall board by utilizing woods of the types above set 65 forth.

When hard woods which have a dense formation, comprising relatively short fibres, are used alone in the manufacture of wall board it is preferable to lightly cook such wood either with 70 plain water or with a chemical solution, such as, for example, a mild caustic or acid solution, before grinding or disintegrating. The grinding or disintegrating process should be so conducted as to give relatively short and properly hydrated fibres, which will form a pulp having a degree of freeness that will permit proper formation of a wet board cake on a board forming machine.

*Example 1.*—As an example of one method by which suitable hard wood pulp may be produced, 80 the hard wood is prepared in the usual manner by chipping or reducing in other manners to suitable dimensions to permit proper contact, circulation, and penetration of the cooking liquor. The wood in this form is next cooked either with 85 plain water or with a mild caustic or acid solution for from 1 to 6 hours. The cooking may be conducted either in an open vessel or in a closed vessel under pressure. When the wood has been properly cooked it is next transferred to a grinding or reduction mill, which may be of a more or less conventional form such as, for example, a Bauer grinding mill, a Bird refiner, a rod mill, a stone wood pulp grinder, a hammer mill, a shredder, disintegrator, etc.

Wall board, when formed from hard wood pulp alone, made in accordance with the above process, is in the form of a relatively light, firm and stiff sheet having good nail-holding properties and a relatively high insulating value. This sheet, however, while suitable and preferable for certain uses, is inclined to be brittle and relatively inflexible and modifications are necessary for board to be used in other fields.

For the purpose of obtaining a greater degree of flexibility of the sheets formed from hard wood pulp, it is desirable to mix with the hard wood pulp varying proportions of soft wood pulp, or soft wood pulp mixed with other vegetable fibres 110

- having characteristics which will give to the board increased strength and flexibility.
- Example 2.*—As an example of this method of producing pulp, the hard wood is ground or disintegrated, either with or without the preliminary cooking, the grinding or disintegrating being so conducted as to produce relatively short, hydrated fibres. The soft wood is ground or disintegrated without cooking so as to produce relatively long fibred pulp, after which the hard and soft wood pulps are intermixed in varying proportions. The intermixed pulp is then delivered to the board forming machine and formed into board. The soft wood fibres, being of relatively greater length than the hard wood fibres bring to the board an increased degree of flexibility and strength which, for some purposes, renders it more easily handled with less danger of breaking when bent. While mixtures of one part each of hard and soft wood pulps on the bases of dry fibre is found suitable, these proportions may be varied from a mixture containing a small percentage of soft wood and a high percentage of hard wood to a mixture containing a small percentage of hard wood and a high percentage of soft wood without seriously affecting the strength and flexibility of the product.
- The hard and soft wood pulps which are to be intermixed should preferably, but not necessarily, vary in freeness to get the desired results. The hard wood pulp may be either more or less free than the soft wood pulp and this variance of freeness may be extended considerably in either direction so long as the freeness of the mixture is within certain limits defined by the proper functions of the particular forming machine used. The freeness of each pulp can and will be varied depending on the proportions of the two woods used in mixture.
- In order to define the degree of freeness suitable for the pulp mixture, for the purposes herein set forth, the following data is given. A cylindrical vessel having a diameter of  $9\frac{1}{8}$  inches, and a height of 8 inches provided with a 60 mesh screen at its bottom is used for the reception of the suspended pulp. The mixture is made up so as to give a consistency of substantially 1%. This receptacle is then filled to the top with the pulp and water mixture at a temperature of approximately  $70^{\circ}$  F. The bottom of the receptacle is provided with a suitable arrangement for attaching a suction pump thereto and after the stock has been poured in, it is subjected to a suction equivalent to approximately 26 inches of mercury. For the stock to have a suitable freeness it should be such that substantially all the water will be drained or sucked out in about 65 seconds. However, the time in seconds for draining may vary from 50 to 110 without materially affecting the formation of the board on the board forming machine. Certain of these factors may vary within substantial limits without affecting the formation of the board on the machine. Thus if the freeness as represented in seconds is altered so that the stock is slower, the temperature and suction could be correspondingly changed to compensate for the difference in freeness.
- Example 3.*—The hard wood is ground or disintegrated, as in Example 2, either with or without preliminary cooking and the soft wood to be mixed therewith is first cooked from 1 to 6 hours and then ground or disintegrated. The pulps thus formed are then mixed in proportions, such as given above under Example 2, so that the stock has a suitable freeness as previously explained, after which it is formed into board in the usual manner.
- Example 4.*—The hard wood and soft wood pulps are prepared as in the above examples by 80 grinding or disintegrating, either with or without preliminary cooking. These pulps are then mixed and to the mixture is added a quantity of from 5% to 25% of true chemical pulp such as kraft or sulphite, or pulp mill tailings, screenings, or suitably prepared vegetable fibres such as cornstalks, straw, grasses, etc. Pulp characterized by the foregoing list being composed of relatively long fibres or fibre bundles makes possible the production of a suitable board even 90 when the hard and soft wood pulps have a preponderance of relatively short fibres and fibre bundles.
- Example 5.*—The hard wood pulp is prepared as in the above examples by mechanical reduction either with or without preliminary cooking and, instead of mixing in a quantity of ground soft wood, the hard wood pulp may be mixed alone with from 5% to 25% of true chemical pulp, or pulp mill tailings, screenings or suitably prepared vegetable fibre. This mixture is then formed into a sheet in the usual manner. In this production the hard wood pulp furnishes a board having good insulating qualities by reason of its porous structure and the added pulp, being composed mostly of long fibres or fibre bundles, acts to effectively bind the hard wood fibres together and gives the board more strength and flexibility and prevents it from being too brittle.
- The pulp mixtures as described in the above given examples are mixed with water in the usual manner to get the desired consistency and are formed into board on any suitable board forming machine such as the Oliver type or the Four-drainer type. If desired, the pulp mixture may be suitably sized to render it water proof.
- The use of the term "fibre" or "fibres" in this specification and in the claims is intended not only to refer to the individual fibres but also to refer to pulp particles which are in the nature of fibre bundles.
- The use of the term "board" in this specification and in the claims is intended to cover any form of article into which the pulp is made without regard to the thickness or other dimensions thereof.
- The present invention thus provides a wall board or analogous composition, in which varying proportions of hard wood pulp and soft wood pulp may be utilized and in which the proportions of either pulp may predominate if desired. Where flexibility and high strength are necessary considerations these characteristics of the board may readily be increased by the use of 135 long fibred soft wood pulp or by the addition of long and tough fibred chemical pulp, tailings, screenings or vegetable fibres. The freeness of the stock is so controlled that a board of a maximum strength may be formed with a minimum 140 amount of time on an ordinary board forming machine. The product thus produced is of a generally open porous construction, having relatively high insulating value, with good nail-holding qualities and is relatively easy to cut and 145 handle without undue danger of breakage during handling.
- Having described my invention, I claim:
1. A fibre board of substantial thickness, high insulating value and cellular structure, comprising

ing a mixture of relatively short, hard wood fibres from the group of woods:—oak, gum, tupelo, hackberry, magnolia, elm, maple, birch, beech, and relatively long, soft wood fibres from the 5 group of woods:—cypress, cottonwood, willow.

2. A fibre board as defined in claim 1 in which

the hard and soft wood fibres are in approximately equal proportions.

3. A fibre board as defined in claim 1 in which the hard wood fibres are lightly cooked, and the soft wood fibres are uncooked.

80

CARROLL E. CARPENTER.

|    |  |     |
|----|--|-----|
| 10 |  | 85  |
| 15 |  | 90  |
| 20 |  | 95  |
| 25 |  | 100 |
| 30 |  | 105 |
| 35 |  | 110 |
| 40 |  | 115 |
| 45 |  | 120 |
| 50 |  | 125 |
| 55 |  | 130 |
| 60 |  | 135 |
| 65 |  | 140 |
| 70 |  | 145 |
| 75 |  | 150 |